

## UNITED STATES PATENT OFFICE

2,169,970

## DISAZO DYESTUFFS

Wolfgang Alt and Hans Krzikalla, Ludwigshafen-on-the-Rhine, Germany, assignors to General Aniline Works, Inc., New York, N. Y., a corporation of Delaware

No Drawing. Application October 20, 1938, Serial No. 236,034. In Germany November 19, 1937

5 Claims. (Cl. 260—184)

The present invention relates to disazo dyestuffs, a process of producing same and a process of dyeing textile materials therewith.

We have found that disazo dyestuffs having valuable properties are obtained by causing diazo compounds of aromatic amines to react with ortho-hydroxy-aryl carboxylic arylides containing at least one sulfonic acid group in the arylide portion, which corresponds to the following formula



wherein the Ar stands for arylene radicles, and wherein B<sub>1</sub>, B<sub>2</sub> and B<sub>3</sub> stand for phenylene radicles.

20 Arylides of this type may be prepared for example by reacting two molecular proportions of an ortho-hydroxy-aryl carboxylic acid, e. g. 2-hydroxynaphthalene - 3 - carboxylic acid, their chlorides, their ortho-acyloxy chlorides or their esters with one molecular proportion of an N,N'-di-(aminophenyl)-diamino-benzene sulfonic acid corresponding to the general formula



30 wherein B<sub>1</sub>, B<sub>2</sub> and B<sub>3</sub> represents phenylene radicles at least one of which contains a sulfonic acid group. These diamines may be prepared by condensing phenylene-diamines, e. g. para- or metaphenylene diamine or toluylene diamines, 35 with para- or orthonitrochlorbenzene sulfonic acids which may be further substituted for example by alkyl or alkoxy groups or additional

acid and 7,8-benzocarbazole-Bz.3-hydroxy-2-carboxylic acid.

As diazo components for the process according to this invention there may be mentioned the usual amines employed in the preparation of azo dyestuffs, in particular those not containing solubilising groups, such as aniline, nitroaminobenzenes, nitroaminophenols, aminodiphenylamines, amino-azo-benzenes, which may also contain further substituents, such as halogen or 5 alkyl, fluoralkyl, alkoxy, alkylsulphone or sulphonamide groups. Since the azo dyestuffs prepared with the aid of these diazo components are usually difficultly soluble or insoluble in water, it is preferable for the purposes of textile dyeing 10 to prepare the dyestuffs on the fibre. In this case it is preferable to proceed by applying the said orthohydroxyaryl carboxylic acid arylides to the fibre and developing them thereon by treatment with diazo compounds. 15

The coupling components have affinity for animal fibres and they also go onto vegetable fibres. It is, therefore, possible to produce on mixtures of different fibres, as for example on mixed yarns or mixed fabrics, especially those of wool and 20 regenerated cellulose (staple fibre) very fast dyeings, exceptionally level on both kinds of fibres. 25

The following example will further illustrate how our invention may be carried out in practice but the invention is not restricted to this example. 30

## Example

35 A mixed fabric of 50 per cent of wool and 50 per cent of staple fibre (viscose silk) is treated for an hour at 60° C. in a bath with a bath ratio of 1:20 with 3 per cent of the disodium salt of the composition:



45 halogen atoms, and reducing the dinitro compounds to form diamines.

For the preparation of the arylides there may be mentioned in particular 2-hydroxynaphthalene-3-carboxylic acid, and also other ortho-hydroxy-carboxy compounds capable of coupling, as for example 2-hydroxy-6-methoxynaphthalene-3-carboxylic acid, 2-hydroxyanthracene-3-carboxylic acid, 2-hydroxytriphenylene - 3 - carboxylic acid, 3-hydroxydiphenylene-oxide-2-carboxylic acid, 2-hydroxycarbazole - 3 - carboxylic acid, 2-hydroxycarbazole - 3 - carboxylic

45 with an addition of 50 per cent of sodium sulphate (percentages being with reference to the weight of fibres). After powerful rinsing with cold water, the bottomed fabric is treated for half an hour at room temperature in a neutral solution of the diazo compound of 4-amino-3-50 methoxydiphenylamine or 4-amino-4'-methoxy-diphenylamine. The dyed fabric is then treated for half an hour at 70° C. in an aqueous bath containing from 1 to 5 grams of soap per litre. A navy-blue dyeing of excellent fastness to wash- 55

ing and very good fastness to light which covers uniformly both kinds of fibre is thus obtained. Dyeings on wool or silk or on mixtures of both may also be prepared in the same way. By using 5 4-benzoylamino-2,5-diethoxy-1-aminobenzene instead of the said diazo component, a fast blue dyestuff is also obtained; by using 4-chlor-2-aminodiphenyl ether a red dyestuff is obtained.

Instead of the above described arylide there 10 may be used as coupling component the arylide of the formula:



When developing it with diazo compounds, well 20 covered brown, greenish black or black dyeings may be obtained.

What we claim is:

1. A process of producing disazo dyestuffs which comprises coupling diazo compounds of aromatic amines with orthohydroxy-aryl carboxylic arylides containing in the arylide portion at least one sulfonic acid group and corresponding to the general formula



wherein Ar stands for arylene radicles, and wherein B<sub>1</sub>, B<sub>2</sub> and B<sub>3</sub> stand for phenylene radicles.

40

2. A process of producing fast dyeings on 45 tile material which consists in applying to said



55 material an orthohydroxyl-aryl carboxylic arylide containing in the arylide portion at least one

sulfonic acid group and corresponding to the general formula



wherein the Ar stands for arylene radicles, and B<sub>1</sub>, B<sub>2</sub> and B<sub>3</sub> stand for phenylene radicles, and converting said arylide into a disazo dyestuff by 10 treatment with diazotized aromatic amines.



3. Disazo dyestuffs corresponding to the general formula



wherein the Ar stands for arylene radicles, and wherein B<sub>1</sub>, B<sub>2</sub> and B<sub>3</sub> stand for phenylene radicles and wherein X stands for an aryl radicle.

4. Disazo dyestuffs corresponding to the general formula



wherein X stands for an aryl radicle.

5. The disazo dyestuff corresponding to the 45 formula



wherein X stands for the radicle of a methoxy- 55 diphenylamine.

WOLFGANG ALT.  
HANS KRZIKALLA.